

Jan. 23, 1934.

A. KRONSTEIN

1,944,562

MANUFACTURE OF INSULATING MATERIAL

Filed March 13, 1928

Fig. 1.



Fig. 2.



Fig. 3.



Fig. 4.



Inventor:  
Abraham Kronstein  
per:  
Dr. Adolf Zinnermann  
Attorney.

## UNITED STATES PATENT OFFICE

1,944,562

## MANUFACTURE OF INSULATING MATERIAL

Abraham Kronstein, Karlsruhe, Germany, assignor to the firm Electra-Lackwerke G. m. b. H. System Dr. Kronstein, Karlsruhe, Germany

Application March 13, 1928, Serial No. 261,417, and in Germany July 2, 1927

7 Claims. (Cl. 154—2.6)

This invention refers broadly to electrically insulating material, and it is intended among other important objects to devise means of improving the quality and the life of such products, 5 to increase their resistibility both against electric influences as well as against the action of moisture and heat and atmospheric agents, and to generally improve and facilitate the process of manufacture. In the electric arts it has been 10 common to mainly employ rubber and the so-called linoxyn, that is to say the oxidation product obtained by the action of air upon linseed oil, preferably heated linseed oil, and oil varnish, as insulating materials, besides other substances, 15 all such insulating compounds being usually combined with other insulating agents; such as paper, linen, silk and equivalent means, all of which possess a higher degree of mechanical strength and resistibility. The manufacture of 20 these products has been mostly carried out by applying a solution of the rubber or of the linoxyn unto the material of higher mechanical resistibility, and by then drying the coating obtained. This drying procedure must be carried out by 25 oven—or furnace—heat or by means of hot air, in order to completely remove the solvent, and to produce a dry and solid layer. In the case of the linoxyn, insulating oil-varnish has been 30 usually employed as the starting material for the manufacture, the procedure being such that the linoxyn has been generated only in contact with the carrier base, such as silk, linen, paper and the like. With this manner of operation the 35 nature of the fibre of the carrier is very injuriously affected by the heat employed, so that the strength and permanency of the material are considerably reduced. After a certain time various defects are presenting themselves which are generally designated as collapsing phenomena, and the insulating material as a result thereof becomes brittle, and the insulating qualities are decreased with the additional drawback that the material is gradually losing its 40 resistibility against the entrance of moisture.

45 Now, these difficulties are overcome in accordance with this invention by combining an electrically insulating material, such as for instance rubber—solution, solutions of artificial resins, insulating varnish, that is to say, so-called oil-varnishes, including the linoxyn, or so-called “zapon”—varnishes, that is to say, celluloid-varnishes, solutions of nitro-cellulose with or without camphor, or solutions of celluloid in acetone, amyl-acetate, ether or the like, including solutions of acetyl-cellulose or of nitrocellulose generally, electrically insulating adhesive varnish, including artificial resins or the like with a carrier base or layers comprising a modification of cellulose which is free from fibrous constituents, and is commonly known in the trade as so-called 60 pure, mostly glycerine-containing cellulose as distinguished from the carriers consisting of cellulose-esters as heretofore employed. These carriers as disclosed by the previous art are objectionable on account of their becoming decomposed by friction and by the influences of the electric currents and electro-magnetic fields which cause them to liberate their acid constituent and to swell up and assume a porous condition. It should also be noted that the 65 cellulose-compounds containing nitrated constituents are inflammable by short-circuiting. Then, in the employment of these and similar carriers for electric insulating and allied purposes it is of paramount importance to avoid 70 the presence of fibers in the insulating units, inasmuch as impregnated fibers are subject to ageing and become brittle, and even the slightest amount of projecting fibers is liable to produce 75 sparking. The suggestions contained in the previous art, so far as I am aware, have failed to produce insulating units from cellulose-material which are both heat-proof as well as non-swelling and free from fibers. In view thereof 80 I have entirely discarded the use of cellulose-esters and instead thereof my invention provides for the use of substantially pure homogeneous and not esterified cellulose as obtained by the solidification of more or less dissolved cellulose. Such kinds of cellulose are for instance 85 designated by various fancy names, such as “Cellophane”, “Transparit”, “Gaudophil” and others, all these substances or compounds being obtained from cellulose by treatment with carbon-disulfid and soda-liquor or caustic soda and 90 containing a certain amount of glycerine which makes them transparent or translucent. The cellulose-product by itself is a very poor insulator. Now, I have found in the course of my experiments that by the combination of a carrier 95 base or layers of these cellulose-products with the electrically insulating agents above enumerated it is possible to produce a material which is free from fibres and possesses an exceedingly high degree of electric resistance, and 100 which will retain its valuable properties for an unlimited length of time, and which, moreover, is water-proof and is not affected by high temperatures, so as to be particularly well adapted 105 for use in the electric arts for various purposes. 110

In view of the fact that the product resulting from the combination of materials referred to presents a new composition, free from fibers which is not affected by high temperatures, it 5 becomes possible to combine the cellulose-products with the varnish at high temperatures, without thereby in any way detracting from the flexibility or resistibility of the final product.

While the electrically insulating materials 10 heretofore known and comprising a combination of fibrous material and varnish constitute a film or a membrane of linoxyn through which gases will diffuse, so that they are not adapted to produce a sufficient protection of electric machines 15 against moisture and acid vapors, the product according to my invention is absolutely impermeable for gases and water. The product obtained in the manner described is moreover oil-proof, and the costs of manufacture thereof are nevertheless lower than those of compositions in accordance with the previous methods. This is 20 mainly due to the fact that the cellulose products above referred to, as found in commerce, produce smooth-faced carriers, while in the case 25 of other carriers, such as linen, silk, paper or the like, rather expensive operations were necessitated, in order to cause them to present a smooth outer surface, it being well known that 30 smoothness of surface of the insulating material is an indispensable requirement for the prevention of electric discharges.

The process of manufacture of the insulating material may be carried on in different ways. Thus I may proceed for instance by applying 35 the insulating compound, such as linoxyn, rubber or a rubber-mixture or—compound to one side of the cellulose material, by which means an insulating material or an insulating band or ribbon having any desired degree of adhesiveness 40 and possessing a smooth, hard back surface of cellulose material is obtained which is particularly adapted for use with low voltages. However, it is also possible to coat this material on the other untreated side with the same material 45 or with an insulating material of other qualities, so that a new product is obtained the properties of which may be varied in any suitable manner as compared with the material coated on one side only. Thus it is possible in this manner to 50 impart a higher insulating action to one side of the material than to the other side thereof. By using coats of different thickness on both sides of the carrier bending of the electric insulating units thus obtained is facilitated, the 55 elasticity is vastly increased and all tendencies of cracking of the coating are eliminated. Any desired changes or varieties as regards mechanical properties, resistance, self-induction or capacity of the two coats and as regards other qualities 60 may be produced; or an insulating band or ribbon may be obtained according to this invention which is provided on one side with an adhesive agent, while the other side thereof is highly insulating and accordingly dry and free from adhesive properties.

In the case of insulation being provided on both sides of the article the insulating layers may be of the same or of different thicknesses on both sides.

70 The cellulose-composition according to this invention is free from fibres, and free from ester constituents and accordingly not liable to lose its impermeability by decomposition and it may be employed moreover for the manufacture of 75 finished articles, such as electrically insulating

tubes and other pieces of insulation, which latter may for instance be worked into finished articles by pasting layers of the cellulose composition with a liquid insulating material, such as adhesive insulating varnish, or by a solution of artificial resin or the like, or in any other suitable manner.

80 Much stronger units of insulating material may be obtained by producing the final insulating sheets, blocks or articles from fibreless cellulose-material which has been varnish-coated on one side or on both sides by the pasting together of two or a plurality of such insulating layers or by producing a combination or aggregation thereof in any other suitable manner. These articles will then comprise a large number of superimposed insulating layers by which means the electric resistance becomes exceedingly high.

85 It is also possible, of course, to obtain finished articles from cellulose—compounds free from fibres which possess the final shape of the desired insulating unit, and then convert them into the superior insulating composition and articles by the application of insulating compounds, such as linoxyn or oil-insulating varnish or the like, 90 after having imparted the final shape to such bodies.

95 The invention is illustrated diagrammatically and by way of example on the accompanying drawing in Figures 1 to 4 showing longitudinal 100 sections through pieces of insulating units according to my invention, the cellulose base or a carrier being designated *a* in all of the figures, while *b* and *c* are layers of insulating material, linoxyn or the like, as above set forth and respectively disposed on the two sides of the carrier *a*. In Figure 3 a comparatively thinner layer *d* of a suitable adhesive is arranged at the bottom side of the carrier base *a*. In Figure 4 I have shown 110 diagrammatically an aggregate of superimposed pairs of layers *a* of cellulose with interposed layers of insulating material *b*.

115 It will be obvious and should be understood that variations and modifications are possible as regards the manner of combination of the constituents of the insulating products and articles described, and it is therefore aimed to cover all modifications and embodiments of the principles of the invention, which do not involve a departure from the spirit and scope thereof, as defined 120 in the appended claims.

I claim:—

1. As new articles of manufacture electrically insulating units, comprising thin, fibreless, unsaponifiable carrying sheets of viscose-like, solid 130 regenerated cellulose and a coating of solidified linseed-oil oxidation products.

2. As new articles of manufacture electrically insulating units, comprising impermeable, water-proof, thin and fiberless, unsaponifiable carrying sheets of viscose-like, solid regenerated cellulose and a coating of homogenous, rubber-like and stretchable, substantially oil-proof, water-insoluble, organic solid electric insulating material, superficially and firmly united to said 140 carrying sheets.

3. As new articles of manufacture electrically insulating units, comprising impermeable, water-proof, thin and fiberless substantially transparent, unsaponifiable carrying sheets of viscose-like, solid regenerated cellulose and a homogenous coating of solidified linseed-oil oxidation products superficially and firmly adhering to said 146 base.

4. As new articles of manufacture electrically insulating units comprising a thin and fiberless sheet of impermeable, water-proof, solid, viscose-like regenerated cellulose, a comparatively thin coating of solidified linseed-oil oxidation products on one side of said sheet, and a comparatively thick coating of such linseed-oil products on the opposite side of the sheet, said coatings being superficially firmly united to said sheet.
- 10 5. As new articles of manufacture electrically insulating units, comprising a thin and fiberless sheet of impermeable, water-proof, solid viscose-like regenerated cellulose, a coating of solidified linseed-oil oxidation products on one side of said sheet and superficially firmly united thereto, and an adhesive coating on the opposite side of said sheet.
- 15

6. As new articles of manufacture insulating units, comprising a thin and fiberless sheet of impermeable, water-proof regenerated glycerine-containing cellulose and a coating of homogeneous, rubber-like and stretchable, substantially oil-proof and water-insoluble, organic solid, electric insulating material superficially firmly united to said sheet.

7. The method of manufacturing electrically insulating units which comprises coating sheets of solid, viscose-like and fiberless regenerated cellulose at ordinary temperature with linseed-oil oxidation products and causing said products to become firmly united and solidified in permanent contact with the surface of said sheets.

ABRAHAM KRONSTEIN.

20

95

25

100

30

105

35

110

40

115

45

120

50

125

55

130

60

135

65

140

70

145

75

150